

# UNITED STATES PATENT OFFICE.

WOOLSEY McA. JOHNSON, OF HARTFORD, CONNECTICUT.

## CADMIUM-EVOLVING PROCESS.

1,271,172.

Specification of Letters Patent.

Patented July 2, 1918.

No Drawing.

Application filed July 30, 1914. Serial No. 854,169

*To all whom it may concern:*

Be it known that I, WOOLSEY McA. JOHNSON, a citizen of the United States, and residing at Hartford, in the county of Hartford and State of Connecticut, have invented a new and Improved Cadmium-Evolving Process, of which the following specification is a full disclosure.

This invention proposes a treatment capable of deriving from cadmium-bearing materials a greater yield of that metal than has heretofore been commercially attainable and, from a more specific aspect, this invention contemplates a reformation of present methods of deriving zinc from its ores so as to render available a treatment of a differential character which, while effecting a more complete recovery of the cadmium will at the same time realize a more complete yield of the companion metals and values such as zinc, copper, lead and the precious metals.

At the present time, cadmium is commercially obtained as a by-product incidental to the recovery of zinc by the so-called "re-torting" method now in current use, and a predominant characteristic of that method is that the liberation of the cadmium in the ultimately prepared charge ensues mainly coincidentally with that of the zinc. Consequently, the cadmium to a large extent finds its way into the "blue-powder" to form a small constituent element thereof, and this blue-powder is the ultimate source of such cadmium as is now commercially available. Its isolation from the zinc is of necessity accomplished through a rather involved and elaborated treatment and re-treatment of the cadmium-bearing blue-

powder. Much of the evolved cadmium, however, fails to be carried into the blue-powder and accordingly is non-recoverable for the reason that it condenses with the zinc to form a permanent element of the spelter; sometimes in a proportion as high as 2% thereof. The cadmium thus confined by the spelter not only represents a loss directly proportional to the value of the cadmium, but it also impairs the value of the spelter when present in material amounts because it diminishes the adaptability of the spelter

for certain purposes; notably for rolling into sheet zinc.

Now by this invention there is created a process of smelting zinc ores so formulated that, not only will higher yields of zinc and companion metals be obtainable, but the loss of cadmium will also be greatly decreased and its recovery free from zinc and in a form suitable for various purposes will be facilitated.

The primary characteristics of this method may be better revealed by assuming a typical ore-analysis, and then explaining one of the various ways in which it would be treated in accordance with this invention; and illustrating the various typical changes in composition resulting during the progressive stages of this treatment.

Assume a native zinc-cadmium sulfid ore analyzing about as follows:

(A) 27.3% Zn; 0.70% Cd; 2.076% Pb; 14.6% Fe; 4.3% Cu; 3.2% CaO; 10.8% SiO<sub>2</sub>; 31.3% S.

It may be explained that the ore represented by (A) is too high in sulfur for subsequent treatment and it must be prepared by first being subjected to a special roasting or calcining operation. In contra-distinction from the conventional roasting of re-torting practice, this preliminary calcining operation preferably does not eliminate all sulfur and it is so conducted as not to expose the ore for a material length of time to a temperature exceeding 800° C. (as distinguished from the usual 1000° C. conventionally employed) in order that the loss of cadmium in the fume from the roaster will be kept as small as possible.

It should here be explained that, under ordinary roasting conditions and at a temperature of 800° C., CdS is oxidizable to CdO at a sufficient rate or speed of reaction to enable my lower temperature to be used in connection with the limited time-periods commercially available; and it should be further noted that the CdO thus formed may then be reduced by carbon to metallic cadmium (as a gas which changes to cadmium blue-powder) at a temperature of about 730° C., as contrasted with the tem-

perature of  $1040^{\circ}$  C., required for the initial reduction of  $ZnO$  to  $Zn$ .

I have, however, discovered that in the presence of considerable amounts of the usual sulfur-bearing materials the roasting may be conducted to an extent satisfying the needs of the further steps of my process and at a sufficient speed by employing a temperature of about  $800^{\circ}$  C. In other words, instead of forcing the roasting to the point of a practically complete elimination of the sulfur, as is now done with present zinc-retorting methods, I preferably propose so to modify the prevailing roasting step as to leave considerable amounts of sulfur in the ore, say about 5%, and thus avoid the stringent forcing conditions that have heretofore obtained, and which have caused very great losses of cadmium during the roasting operation. It should be explained that cadmium oxid is to a small extent volatile in the sweep of the gases of a roasting furnace and, as this sweep is considerably higher under the higher temperature conditions of conventional roasting, the loss is correspondingly greater due to this cause than in my process in which this step is more moderate. Thus, as a result of my special temperature roast, the above mentioned typical ore would be caused to analyze about as follows:

(B) 31.2%  $Zn$ ; 0.93%  $Cd$ ; 2.3%  $Pb$ ; 17.4%  $Fe$ ; 4.8%  $Cu$ ; 4.0%  $CaO$ ; 14.2%  $SiO_2$ ; 5.9%  $S$ .

The above product (B) has, in a sense an anomalous composition, inasmuch as it is unsuitable either for conventional retorting practice (by reason of its comparatively high content of sulfur) or for economical electric smelting, since its constitution prohibits it from being entirely and completely smelted into slag, matte, fused-bullion, gases and vaporized metal and it, therefore, demands to be modified in composition to a greater or less degree so that its immediate reduction may be accomplished continuously and without undue consumption of current. In this instance, but little modification is demanded, since the above roasted product (B) happens to be about completely self-fluxing since it needs the addition of only about 4% of  $CaO$ , in the form of quick lime, together with about 22% of soft-coal (analyzing 75% fixed carbon, 20% volatile matter and 5% ash); the theoretical carbon requirements being 16.3% for the reduction to sulfids of the  $CdO$ ,  $Fe_2O_3$ ,  $CuO$  and any sulfates. In certain instances, the product at the end of the roasting operation will be of a more pronounced non-fluxing character; thus rendering necessary a more radical reconstruction of its composition by providing it with the necessary amount of carbon

and slagging constituents. In any event, 65 a charge analyzing about as follows is to be obtained from the roasted product:

(C) 24.0  $Zn$ ; .71  $Cd$ ; 1.8  $Pb$ ; 13.4  $Fe$ ; 3.7  $Cu$ ; 6.14  $CaO$ ; 11.3  $SO_2$ ; 4.6  $S$ ; 12.7 70 fixed carbon.

This charge (C) is then subjected to a preliminary heat treatment devised to effect a substantially complete recovery of the cadmium without appreciably evolving zinc, 75 and at the same time be adapted to effect a metallurgical alteration (as by reducing  $Fe_2O_3$ ,  $CuO$  and sulfates) in the charge of such a character as will particularly adapt 80 it for an economical electric-furnace treatment. Suitable amounts of iron, silica, or old slag, lime or the like may be added to the product (B) so that after the preliminary cadmium-evolving heat-treatment the resultant product will be constituted to smelt 85 with a production of enough slag to keep the furnace open and free working.

(D) 25.7%  $Zn$ ; 0%  $Cd$ ; 1.8%  $Pb$ ; 14.3%  $Fe$ ; 3.96%  $Cu$ ; 6.6%  $CaO$ ; 13.1%  $SiO_2$ ; 90 4.98%  $S$ ; fixed carbon.

This cadmium-evolving heat-treatment was carried out under reducing conditions by causing the charge C (which is B, modified 95 as stated) to pass through a suitably constructed furnace such as a muffle-furnace of the Hasencleoeer type so as to pre-heat and pre-reduce the "mix."

This intermediate or cadmium evolving 100 furnace is constructed to permit the temperature to be controlled so as to prevent it from rising above  $1000^{\circ}$  C. for any preventable periods and for enabling it to be maintained above  $800^{\circ}$  C. The charge, which 105 preferably contains soft coal or other carbonaceous material of such character as to evolve reducing gas at the temperature of the furnace, is caused to feed into the furnace and to be therein subjected to the temperature thereof for such a time as will be adequate to effect an evolution of the cadmium in the form of cadmium blue-powder. Preferably the reduction will be effected 110 in the presence of a stream of suitable reducing gas, such as will be evolved by the soft coal or other volatile carbonaceous material preferably used in the charge, so as to sweep the cadmium blue-powder into a 115 suitable condenser. By conducting this operation under the conditions specified, a reaction will ensue and the cadmium will be isolated from the zinc (which remains un-reduced and unvolatilized and confined to the charge) and a further important constitutional alteration will take place in the charge. That is to say, the iron oxids, in 120 the presence of the carbon and at the tem-

perature of the furnace and during the time of the treatment, will to a material extent be metamorphosed and converted into a sensitively reactive metallic or semi-metallic 5 condition, enabling it to coöperate in the subsequent step in promoting the reduction of the zinc oxid and effect an important and substantial economy in the consumption of the electric-furnace.

10 The "cadmium blue-powder" (product E) evolved analyzing 75% Cd during the execution of this step, will be collected in "prolongs" suitably arranged and further refined in any suitable manner, such as that 15 conventionally practised, but it is noteworthy that this blue-powder is (in contradistinction from that derived as a result of the conventional retorting practice) characteristically free from substantial amounts of 20 zinc. It is also noteworthy that the amount of cadmium recovered at this point greatly exceeds that recoverable by the retorting method, inasmuch as the loss during the roasting operation is reduced to a minimum 25 and all the cadmium is extracted at a point in advance of the evolution of the zinc so that it is prevented from entering either the spelter or the zinc-blue-powder.

The typical ore that which was utilized 30 for the purpose of revealing the more fundamental characteristics of this invention is of course to be understood as exemplifying a variety of ores. Certain modifications and refinements are contemplated in the case of 35 special ores. For example when the ore contains large PbS or PbSO<sub>4</sub> which would be reduced to PbS (under pre-heating conditions) the volatile emanations would be passed through an apparatus for precipitating 40 the metallic values, as for instance by passing the emanations through settling chambers or through a small bag house or through a Cottrell electrostatic apparatus so as to obtain a precipitate or condensate 45 containing considerable PbS and PbSO<sub>4</sub> (the latter caused by oxidation of PbS) as well as metallic cadmium. This will better be understood by explaining that lead-sulfid (PbS) has an appreciable vapor tension at 50 800 degrees C. to 900 degrees C. so that the resultant vapor existing in the pre-heating furnace will be swept away in the current of gas along with the cadmium vapor and, when there is much PbS in the mixture 55 (say from 10% to 15%) the precipitated cadmium blue-powder will be contaminated by the lead. A consequential saving of the lead that otherwise would be lost is thus effected because this lead would otherwise 60 have mixed with and deteriorated the spelter and never be isolated therefrom, whereas when concentrated in the cadmium blue-powder, it will be recovered during the subsequent isolation of the cadmium.

Under such conditions it is proposed to 65 subject the contaminated cadmium blue-powder to a 10% solution of sulfuric acid so as to dissolve the cadmium sulfate and relieve an insoluble residue lead sulfate which may be isolated by a filter press and 70 reduced during the electric smelting operations. The cadmium may be recovered from the filtrate in any suitable manner, as by electrolyzing it in a nearly neutral state in vats, using a lead-anode and forming cathodes of pure cadmium which can then be melted into commercial form. As the cadmium is present in a finely divided form in the condensate it will readily react with the diluted acid, so the control of the acidity of 80 the solution is almost automatic.

The de-cadmiumized residue (product D) may now be treated in any appropriate manner to recover its metallic values. It may be explained, however, that the foregoing treatment was devised not only to isolate the cadmium values but at the same time to condition the residue for a continuous electric smelting of the zinc in accordance with my U. S. Patent #868345. On the other hand, 90 if circumstances are such that it would be more profitable to produce a non-slaggering mixture with a corresponding conditioning of the charge, the de-cadmiumized residue could be treated by charging into an ordinary retorting furnace.

In the case instanced, charge D would be passed into a suitably constructed electric furnace and smelted electrically to obtain cadmium-free spelter and cadmium-free 100 blue-powder.

The spelter thus made by electric smelting of this de-cadmiumized product shows on analysis less than 0.01% Cd and is preferable for many purposes.

Having thus revealed this invention, I claim as new the following combination of steps, or of equivalents thereof, and desire to secure the same by Letters Patent of the United States:—

1. A process of the nature disclosed for deriving cadmium from sulfur-bearing ores which consists in preliminarily effecting an incomplete roasting of the ore to reduce the sulfur contained therein to not materially less than about 3%, and thereafter subjecting the partially-roasted material to reducing conditions to reduce and evolve cadmium contained therein.

2. A process of the nature disclosed for 120 deriving of cadmium from a sulfur-bearing material which consists in preliminarily effecting an incomplete roasting of the material and subsequently subjecting the incompletely-roasted material to reducing conditions in the presence of a current of gas effective to carry off the evolved cadmium vapors.

3. A process of the nature disclosed for 05 differentially reducing a cadmium-zinc bearing material; comprising obtaining the material with a considerable sulfur-content and then subjecting the said sulfur-bearing material under reducing conditions to a temperature sufficiently high to evolve cadmium vapors but too low to evolve zinc vapors.
4. A process of the nature disclosed for 10 treating a sulfur-bearing zinc-cadmium product which comprises subjecting it to a prolonged treatment under reducing conditions at a temperature below 1000° C. to evolve cadmium blue-powder without effecting a substantial reduction of the zinc, and then subjecting the residue while containing a material amount of sulfur to a temperature exceeding 1000° C. under reducing conditions to evolve condensable zinc vapors.
5. A process of the nature disclosed for 15 differentially deriving cadmium and zinc from a sulfur-bearing product containing the same, which comprises the step of preliminarily and incompletely desulfurizing the product and then subjecting the partially desulfurized product for a prolonged period to a current of gas under reducing conditions until the greater proportion of the cadmium present has been reduced and vaporized.
6. A process of the nature disclosed for 20 continuously producing cadmium from material containing not less than about 3% of sulfur consisting in subjecting the sulfur-bearing material under reducing conditions to a temperature sufficiently high to effect an evolution of cadmium blue-powder and too low to effect an evolution of the zinc.
7. A process of the nature disclosed for 25 deriving cadmium from sulfur-bearing ores which consists in preliminarily effecting an incomplete roasting of the ore at a moderate temperature to eliminate the greater amount of sulfur contained therein, then discontinuing the roasting before the sulfur content is reduced sufficiently to permit the ore to be retorted; and then subjecting the partially-roasted material to reducing conditions to liberate the cadmium contained therein.
8. A process of the nature disclosed for 30 deriving of cadmium from a sulfur-bearing material which comprises the preliminary step of incompletely eliminating sulfur from said material and the subsequent step of subjecting the material while containing considerable amounts of sulfur to reducing conditions in the presence of a current of gas effective to carry off the evolved cadmium vapors.
9. A process of the nature disclosed for 35 differentially obtaining cadmium and zinc from sulfur-bearing material contained in the same, consisting in first largely but not wholly reducing the sulfur-content of the material; then subjecting the incompletely desulfurized material under reducing conditions to a temperature effective to evolve cadmium vapors but ineffective to reduce zinc vapors.
10. A process of the nature disclosed for 40 treating unsmelted ores containing Cd and Zn which comprises first reducing CdO to Cd at a temperature below the reduction temperature of zinc oxid; evolving same in a gaseous condition; collecting same in a condenser; then immediately treating the de-cadmiumized residue at a materially higher temperature to make a spelter containing a trace only of Cd.
11. A process for conditioning ores to 45 yield cadmium-free zinc which consists in preparing a mixture of ore and solid carbon having the capacity of innately generating non-oxidizing gas, by mixing with carbonaceous material undistilled ore analyzing at least 30% zinc and less than 1% cadmium, and then propelling said mixture through a heated air-excluded zone at a temperature less than that required to reduce zinc-oxid and sufficient to reduce all of the cadmium- 50 oxid.
12. A process for preparing cadmium-free 55 zinc-gas which consists in first roasting the ore to oxidized metallic sulfids, then causing the ores in the presence of a reducing agent to pass through a zone heated to a temperature not exceeding 1000° C. and not less than 800° C. whereby all particles of said ore will be exposed to a temperature not exceeding 1000° C. whereby all of the 60 cadmium may be expelled as a metallic vapor; and then subjecting said preheated ore to zinc reducing conditions at a temperature above 1000° C. to evolve zinc-gas.
13. A process for preparing cadmium-free 65 spelter which consists in first roasting the ore to oxidized metallic sulfids, then causing the ore in the presence of a reducing agent to pass through a zone heated to a temperature not exceeding 1000° C. and not less than 800° C. whereby all particles of said ore will be exposed to a temperature not exceeding 1000° C. whereby all of the 70 cadmium may be expelled as a metallic vapor; and then subjecting said preheated ore to zinc reducing conditions.
14. A process for conditioning ores to 75 yield a cadmium-free zinc which consists in preparing a mixture of ore and solid carbon having the capacity of innately generating non-oxidizing gas, by mixing with carbonaceous material undistilled ore analyzing at least 30% zinc and less than 1% cadmium, and then propelling said mixture through a heated air-excluded zone at a 80 temperature less than that required to reduce zinc-oxid and sufficient to reduce all of the cadmium- 85 oxid.

15. A process for obtaining cadmium from spelter or from ores bearing zinc and cadmium which consists in first roasting the ore; then causing the ore to pass through a  
5 zone heated to reducing conditions at a temperature below 1000° to expel the cadmium as a metallic vapor and then subjecting the product to zinc reducing conditions.

In witness whereof, I hereunto subscribe my name, as attested by the two subscribing witnesses. 10

WOOLSEY McA. JOHNSON.

Witnesses:

DELOS G. HAYNES,  
B. COOKE.